

March 23, 1954

E. J. HICKOX

2,672,978

## METHOD OF MAKING ADHESIVE TAPE

Filed Dec. 28, 1950



100-1000  
Inventor  
Elmer J. Hickox  
by  
Willis Hardman & John  
his attorneys

Patented Mar. 23, 1954

2,672,978

# UNITED STATES PATENT OFFICE

2,672,978

## METHOD OF MAKING ADHESIVE TAPE

Elmer J. Hickox, Warren, Ohio, assignor to General Motors Corporation, Detroit, Mich., a corporation of Delaware

Application December 28, 1950, Serial No. 203,127

3 Claims. (Cl. 206—59)

1

This invention relates generally to the problem of wrapping of an article with tape or to the wrapping of a group of elements with tape to hold such elements assembled together, for example, to the taping of wires to form an assembly commonly known as wiring harness, such as used in automotive vehicles for connecting the generator with the storage battery and other current consuming devices, and more particularly to a method of making an adhesive tape which is suitable for this purpose.

Taping has previously been effected by the use of pressure sensitive tape, known as friction tape, obtained in rolls, the convolutions of which adhere to such extent that, when the peeling off of the free end is started, the weight of the roll can be supported by the free end without causing the roll to unwind. The free end portion having been pressed against the bunched wires so that the unwound roll may be supported by the wire, taping is continued by tossing the roll about the wires. One variety of friction tape which can be obtained is a thermoplastic material such as Vinylite, which has been prepared with an adhesive surface so that the convolutions of a roll of such tape will adhere together.

The primary object of this invention is to provide a method of and apparatus for making a suitable tape which can be employed to wrap the wires of a wiring harness or other elements, from sheets of a thermoplastic material, to the surface of which no adhesive compound has been applied and the surface of which has not been treated in any way. According to the present invention, this object is accomplished by unwinding a sheet of suitable thermoplastic material from a supply roll, slitting the material as it is unwound from the supply roll to form strips of whatever width may be desired and simultaneously winding such strips on hollow cores of paper or other suitable material while the strips are under tension, so as to provide rolls of tape of a size suitable for handling and in which the convolutions of tape are under appreciable tension.

A quantity of these rolls are placed in properly spaced relation on rods which are placed upon a rack in such spaced relation as will enable the rolls to be heated most uniformly. The loaded rack is placed in a suitable heating chamber and the rolls of thermoplastic strips are heated. When heated at the proper temperature and for a sufficient period of time, the surface of the tape becomes sufficiently adhesive to cause the adjacent convolutions of each roll of tape to adhere so as to permit the wrapping of the tape around the wires of a wiring harness or other elements to be carried out in the manner described above, the tape in the roll being sufficiently adhesive to support the roll of tape without permitting it to unwind.

After the rolls of tape have been heated at the proper temperature for the necessary period

2

of time, the heating means is rendered ineffective, the heating chamber is opened and as soon as the temperature therein drops sufficiently, the racks holding the rolls of tape are removed and the rolls are cooled in the room to room temperature.

There are various thermoplastic materials which can be used in carrying out applicant's method and while the heating of the rolls of tape is preferably effected by use of steam, a hot air oven can also be used and, in fact, actually has been used with satisfactory results.

Further objects and advantages of the present invention will be apparent from the following description, reference being had to the accompanying drawings in which a preferred embodiment of an apparatus for carrying out the method of the present invention is shown.

In the drawings:

Fig. 1 is an end view of a rack loaded with rolls of tape to be heated and shown within a circle representing the inside wall of a steam heating chamber.

Fig. 2 is a fragmentary side view of the rack showing some of the rolls of tape supported thereon.

The apparatus for slitting a sheet of suitable material into strips of the desired widths as it is drawn from a supply roll and for simultaneously forming rolls of the strips so formed is not shown herein and any suitable apparatus for unwinding a sheet of thermoplastic material from a supply roll slitting such material into strips of suitable width and winding such strips into rolls while maintaining the strips of material under suitable tension can be used. In other words, the specific construction of the apparatus which is employed to form the rolls of tape is not material and not a part of the present invention. In carrying out applicant's method, the rolls of tape as formed by some suitable apparatus are adapted to be placed on a rack which is movable bodily into a heating chamber in order to effect the desired heating of the rolls of tape supported therein, such rack being described hereinafter.

The reference numeral 10 designates the rack in its entirety and such rack comprises angle iron end frames 11, joined at their lower ends by angle irons 12 which are connected by angles 13. At the top, the frames 11 are connected by two parallel angle irons 14 which are connected with notched blocks 15 which are adapted to receive chain hooks of a hoist for moving the rack. The frames 11 support a plurality of vertically spaced angle irons 16 to each of which is welded a bar 17 having notches 18 for receiving rods 19 which are adapted to support rolls of tape designated at 20 and which, when mounted on the rods 19, are spaced apart a suitable distance. The angle irons 16 prevent any appreciable endwise movement of the rods 19 so that they will not be disengaged from the supporting notches 18 when the rods are

placed on the rack, and the notches are so spaced longitudinally of bars 17 that when all of the notches are occupied by bars 19 the rolls 20 will be located in rows positioned as indicated in Fig. 1.

As already indicated, the rolls of tape 20 are formed by winding strips of thermoplastic tape under tension, as they are received from a sheet slitter, upon hollow cores or tubes 20c of paper or other suitable material, which are placed on and rotated by a winding mandrel which is rotated to draw the thermoplastic material from a supply roll and to effect the slitting of the sheet of material carried by the supply roll into tape of suitable widths.

In forming the rolls, a sheet of suitable material is unwound from a supply roll, is slit into strips of suitable widths as it comes off the supply roll and the strips of tape so formed are wound into rolls. The apparatus employed is provided with some suitable means to place the tape under tension as the rolls are formed. The tension on the tape as the rolls are formed is enough to slightly elongate the material during the formation of the rolls so that after the rolls are formed the tape tends to contract, thus increasing to some extent the compression between adjacent convolutions of the rolls. Of course, the greater the elongation, the greater will be the compression force which is created. It has also been found that there is some variation in this force, it being greater some distance within the roll than near the finish end, but this variation is not sufficient to be of any material importance.

Also there is some variation in tension of the tape in rolls formed from different sheets of material. For example, the material in one supply roll may have a smoother surface than that in another and the roll of smooth material unwinds less easily than a roll with rougher material. These variations in tension are not very great, but it has been found that by modifying the time and/or temperature of the heat treatment of the rolls of tape, which will be described later, the effect of any variation in the tension of the tape in the rolls can be substantially eliminated so that a tape of substantially uniform character can be produced.

The tension on the tape during the formation of the rolls is not sufficient to cause any appreciable permanent elongation of the strips of tape, but is always enough to eliminate wrinkles and to bring about the desired degree of adherence between the adjacent convolutions of the rolls to be obtained when the rolls are heated. The winding operation is continued until the rolls have a suitable diameter, for example, a 4 inch diameter for tape  $\frac{3}{4}$  to 1 inch in width, and a  $4\frac{1}{2}$  inch diameter for tape of  $1\frac{1}{4}$  to  $1\frac{1}{2}$  inch width. The inside diameter of the cores 20c on which the strips of tape are wound is such that the cores fit loosely on rods 19 which may be of  $\frac{1}{2}$  inch diameter, for example.

The rack 10, when loaded with the coils of tape to be heated, is elevated by a hoist which is not shown, placed on rollers 21 and positioned within a heating chamber, the inside wall of which is indicated by the circle 22. This chamber may be a steam vulcanizer of conventional type. The door of the vulcanizer is closed when the loaded rack is positioned therein and the steam is then turned on full to the steam controller and a hand valve is opened until steam is seen issuing from the bleeder valves of the vulcanizer. The steam supplied to the vulcanizer is under the control of an automatic control means which limits the tem-

perature to that desired and maintains the temperature at that value. The heating of the rolls can be effected by subjecting them to the effect of steam at  $212^{\circ}$  F. and under no pressure, if the heating operation is carried out for a sufficient period of time and good results have been also obtained if the rolls are heated for a somewhat lesser period of time at a steam pressure of 2 to  $4\frac{1}{2}$  pounds and temperatures in excess of  $212^{\circ}$  F., for example  $218^{\circ}$  to  $225^{\circ}$  F. However, the best and most uniform results have been secured by subjecting the rolls in the vulcanizer to the action of steam at atmospheric pressure and  $212^{\circ}$  F. for a period of approximately 15 minutes, then raising the steam pressure to a pressure of 2 to 4 pounds, with consequent raise in temperature, and continuing the heating cycle for approximately another 15 minutes. This part of the cycle may be varied to some extent when different thermoplastic compounds are used so as to produce substantially the same degree of adhesion with the different compounds.

As soon as the heating operation is completed, the steam is shut off and the drain valve of the vulcanizer is opened and as soon as possible after the steam pressure has dropped to zero the vulcanizer is opened, the rack with the heated rolls thereon is removed from the vulcanizer so that the tape rolls may be ultimately cooled by the surrounding atmosphere to room temperature. When the rolls are sufficiently cooled, they may be removed from the rack and may be used immediately or stored for future use as the surface of the tape remains adhesive for a long period of time, if the rolls of tape are not unwound, although the surface of the tape does not at any time feel sticky or tacky to the touch.

The heating of the rolls of tape can be carried out at even higher temperatures if the heating time is suitably reduced and satisfactory results obtained, but as stated, the best results have been obtained by heating during the first part of the heating cycle at  $212^{\circ}$  F. and during the second part of the cycle at a temperature of  $218^{\circ}$  to  $225^{\circ}$  F. It will be further understood that instead of employing a steam vulcanizer, the loaded rack could be placed in a suitable hot air heating oven heated either electrically, or otherwise, and if such oven is maintained at the proper temperature for the desired period of time satisfactory results could be obtained. In other words, although, according to the present method, the heating of the rolls of tape is preferably effected by use of a steam vulcanizer, the use of the latter is not essential and the heating of the rolls can be effected by other means with good results.

The invention is not limited to the use of any one thermoplastic material. Good results have been obtained with different materials all of which are compounds of polyvinyl chloride resins with certain plasticizers and stabilizing agents. These materials are obtainable on the market and have substantially similar characteristics. For example, one form of such a compound which has been used with very satisfactory results is known to the trade as Vinylite, while another compound of similar character which has also been used with success is known to the trade as Geon. These materials are obtainable in relatively thin sheets for example the Vinylite which has been used has a thickness of .013 and .009 of an inch. Other thermoplastic materials, the surfaces of which will become sufficiently sticky or tacky to cause adjacent surfaces of such material to adhere together with appreciable force

if heated at a suitable temperature for the proper time while such adjacent surfaces are held together under a slight pressure, can be employed. Examples of these are materials which include polyvinyl acetate polyethylene.

When rolls of tape are heated in accordance with the present invention, the tape does not have any pronounced adhesiveness to the surface of the cable in the normal sense, such as ordinary friction tape would have and, therefore, is not adhesive tape in the ordinary sense. However, the tape layers or convolutions stick tight to each other until forcibly unwound from the roll, and it has been found that tape treated in accordance with the present process can be used to wrap the wires of a wiring harness, or for other purposes, as successfully as tape to which some adhesive compound has been applied to the surface, as for example, ordinary friction tape. The principal advantage of the method which constitutes the present invention is to obtain a roll of tape which requires the application of appreciable force to unwind it from the roll which is formed, so that it can be used in the manner in which conventional friction tape is ordinarily used to wrap a wiring harness by tossing the roll around the harness after the free end of the tape is pressed against the harness and without application of any adhesive substance to the surface of the tape. After the wrapping of the harness is completed, the finish end of the tape is usually fixed in place by taking a hitch in the tape and the taped harness may then be placed in a vulcanizer which causes the tape wrapping to be permanently bonded. However, this is not necessary and the tape is sometimes used without carrying out the step of heating to effect bonding.

As already indicated, the tape when wound on the rolls is under some degree of tension. Some tension is necessary in order to cause the adjacent tape turns to adhere to each other when subjected to heat treatment and the greater the pressure, the greater the degree of adhesiveness for any given temperature. It has been actually found that if the tape rolls are supported on edges, the portion of the tape adjacent the support shows greater adhesion, due solely to the relatively slight weight of the roll, than do other portions of the roll more remote from the support, during the heat treatment. Since uniform adhesion in the roll is most desirable, the rolls are supported during the heating operation by rods which run through the cores on which the rolls are wound. Also in order to produce uniformity in the adhesiveness of the tape, it is important to effect uniform heating since variations in application of heat would also produce variations in the adhesiveness of the tape. To this end the rolls are evenly spaced on the supporting rods 19 and the rods are also so spaced that steam can readily pass between all of the rolls of any single row and all of the rows of rolls as well, the rods 19 being arranged about an unoccupied space of substantial size at the center of the heating chamber 22, whereby the steam has more ready access to all of the rolls of tape in said chamber.

While the embodiment of the present invention as herein disclosed constitutes a preferred form, it is to be understood that other forms might be adopted.

What is claimed is as follows:

1. The method of forming a roll of adhesive tape from a thermoplastic material consisting essentially of a plasticized polyvinyl chloride

resin, which includes the step of heating a roll of tape formed of such material while under tension, by subjecting the roll of tape to the heating effect of steam at 212° F., and atmospheric pressure, for approximately 15 minutes and for subsequently subjecting the roll of tape to the heating effect of steam at 2 to 4 pounds pressure and at a temperature of 218° to 225° F. for substantially the same period of time, so as to cause the surface of the tape to become sufficiently adhesive to adhere to the surface of adjacent convolutions with enough force to require application of appreciable force to unwind the tape, the heating temperatures and the time of heating being insufficient to effect fusion of the tape.

2. The method of forming adhesive tape from a thermoplastic material consisting essentially of a plasticized polyvinyl chloride resin, which includes the steps of forming rolls of tape in which the tape is under appreciable tension, from sheets of thermoplastic material of suitable thickness, placing a plurality of such rolls of tape within a closed heating chamber into which steam may be introduced for heating purposes and positioning such rolls within the chamber in such a way that steam may pass adjacent all the rolls and the heating effect thereon is substantially equalized, introducing steam into said chamber at substantially atmospheric pressure for approximately 15 minutes in order to maintain in the heating chamber a temperature of substantially 212° F. and subsequently introducing steam into said heating chamber at a positive pressure of 2 to 4 pounds for approximately 15 minutes in order to maintain in the heating chamber a temperature in excess of 212° F. whereby the surface of the tape is caused to become sufficiently adhesive, to adhere to the surface of the adjacent convolutions of the roll with enough force to require the application of appreciable force to unwind the tape from the roll, the degree of heat to which the tape is subjected being insufficient to fuse the adjacent convolutions of the roll, whereby the roll may be unwound without damage to the tape by the application of sufficient force thereto.

3. As an article of manufacture, a roll of tape in which the adjacent convolutions of the roll adhere in a non-fused relationship sufficiently to withstand unwinding due to the suspended weight of the roll itself, said tape being formed solely of a thermoplastic material consisting essentially of a plasticized polyvinyl chloride resin the surfaces of which are made adhesive by the limited application of heat, said convolutions being under a predetermined pressure due to elastic deformation of said tape during assembly.

ELMER J. HICKOX.

References Cited in the file of this patent

UNITED STATES PATENTS

| Number    | Name            | Date           |
|-----------|-----------------|----------------|
| 1,930,995 | Carroll         | Oct. 17, 1933  |
| 2,093,087 | Lynn            | Sept. 14, 1937 |
| 2,119,163 | Herrmann et al. | May 31, 1938   |
| 2,219,700 | Perrin et al.   | Oct. 29, 1940  |
| 2,395,668 | Kelgren et al.  | Feb. 26, 1946  |
| 2,406,127 | Alfthan         | Aug. 20, 1946  |
| 2,553,816 | Ebel            | May 22, 1951   |

FOREIGN PATENTS

| Number  | Country       | Date         |
|---------|---------------|--------------|
| 440,776 | Great Britain | Jan. 6, 1936 |